

## UNITED STATES PATENT OFFICE

2,215,143

LACQUERED METAL CONTAINER FOR  
FOODSTUFFS

William Clayton, London, England, assignor to  
Crosse and Blackwell Limited, London, Eng-  
land, a British company

No Drawing. Application July 2, 1936, Serial No.  
88,689. In Great Britain July 6, 1935

1 Claim. (Cl. 220—64)

The object of the present invention is to pro-  
vide improved means for internally lacquering tin  
plate containers.

This invention relates to an improved process  
and apparatus for treating metal containers es-  
pecially cans of tin plate.

When food products are preserved in metal  
containers it is frequently necessary to protect  
the metal from attack by coating the metal with  
a lacquer. This coating is usually applied before  
10 the metal sheet is formed into the can and, during  
the mechanical processes necessary to form the  
can, the lacquer film is liable to be ruptured, with  
consequent exposure of the metal and danger of  
15 subsequent corrosion.

According to the present invention I have  
found that a metal container can be very effec-  
tively protected against corrosion by lacquering  
the inside of the said container by depositing the  
lacquer electrophoretically from a lacquer emul-  
20 sion of the oil-in-water type, the deposited film  
being subsequently stoved if necessary.

The lacquers should be light coloured and  
otherwise suitable for contact with foodstuffs,  
25 and asphaltic or pitchy emulsions are thus un-  
suitable.

A suitable emulsion is made from the usual  
ingredients employed for lacquering food con-  
tainers, e. g.

30 Linseed stand oil 175-200 lbs.  
Synthetic resin 100 lbs.  
Mn/Co drier (10:1) 1 lb. of metal as linoleate

Small amounts of a thinner such as turpentine  
35 or white spirit may be added. 30 volumes of this  
lacquer may be emulsified with 70 volumes of  
water containing 0.25% NH<sub>3</sub> by weight as sta-  
biliser.

The cans should be carefully cleaned and free  
40 from grease. When a tinplate can holding 10

fluid ounces forms the anode, an initial current  
of 2 amps. gives an effective deposit in about  
5-10 seconds. After discharging the emulsion  
and washing, the can may be stoved for 30 min-  
utes at 380° F.

The volume of the disperse phase of the emul-  
sion may be as high as 50% and the current  
density may vary between wide limits, the higher  
the current density the greater the rate of dep-  
osition.

When using an aqueous medium which is alka-  
line or oxidising, the invention has an important  
advantage in that as a result of the electrical  
treatment the tinplate gains an anodic protection  
which is manifested in that the subsequent lac-  
quer film no longer shows evidence of sulphide  
10 stains on the plate below. For instance, certain  
tinplates covered with the same lacquer, in the  
one instance electro-deposited and in the other  
with the usual mechanical rolling method, were 15  
made into cans and filled with meat rolls. After  
sterilisation and cooling, the cans were opened,  
and whereas the can internally lacquered in the  
usual way showed marked sulphide staining of  
20 the plate beneath, the can lacquered electrically  
was entirely free from such stain. According to  
the invention, it is therefore possible to employ  
a transparent lacquer for meat products and  
other foods giving off sulphur compounds, in 25  
place of the special lacquers hitherto employed  
containing zinc oxide or other suspended matter.

I declare that what I claim is:

A container for foodstuffs formed from tin  
plate, said container having the inner tin-coated 35  
surface thereof anodically treated to prevent  
staining, and a coating of transparent lacquer  
electrophoretically deposited on and covering the  
inner surface of said container.

WILLIAM CLAYTON. 40